

## UNITED STATES PATENT OFFICE

1,979,188

TREATING NATURAL AND ARTIFICIAL  
FIBERS

Aleidus G. Bouhuys, Enka, N. C., assignor to  
American Enka Corporation, Enka, N. C., a cor-  
poration of Delaware

No Drawing. Original application July 1, 1933,  
Serial No. 678,728. Divided and this applica-  
tion March 23, 1934, Serial No. 717,114

8 Claims. (Cl. 8—5)

This application is a division of my application  
Serial #678,728, filed July 1st, 1933.

The present invention relates to lubrication and  
protection of yarns, threads, filaments, textile  
fibres or the like consisting wholly or partially of  
natural or artificial materials.

After the yarn, thread, or filament has been  
spun or formed and the final product finished,  
it is subjected to considerable physical wear dur-  
10 ing the various knitting, weaving, braiding,  
winding, and other textile treatments or opera-  
tions which it must undergo. Thus, before going  
into various processes such as weaving, knitting,  
braiding, winding, or coning, the yarns, threads,  
15 or filaments are often previously treated for their  
protection with oily treating liquids which form  
a protective film over their surface and which  
have some lubricating properties. So treating the  
yarn, threads, or filaments tends to prevent dam-  
20 age to them during the operations mentioned,  
during which operations the yarn, threads, or  
filaments are usually exposed to comparatively  
high tensions. For economic reasons, such an oil  
treatment of the yarn, thread, or filament is made  
25 while they are in the dry state and during the  
winding operations of the original yarn package.

Coning and winding oils heretofore described  
have the defects that yarns, threads, or filaments  
30 treated with such mixtures require either a thor-  
ough scouring before the yarn, thread, or fila-  
ment is dyed, or the inclusion in the oil of such  
a large amount, (at least over 25%), of sulfonic  
acid salts of mineral oils or other known emulsi-  
35 fying agents as to reduce the lubricating proper-  
ties of the oil to such an extent that it is imprac-  
ticable for commercial use.

Among the objects of the present invention is  
to provide a new and improved method and com-  
position of the character described above for lu-  
40 bricating and protecting yarn, thread, and fila-  
ments, and an improved protected and lubricated  
product.

An improvement of the compositions of the  
present invention over known compositions con-  
45 sists in that, by the admixture of a suitable com-  
bination of alkali metal and organic base soaps  
hereinafter described with mineral oil sulfonic  
acid salts, and mineral oil, a coning oil and/or  
winding oil with much higher lubricating proper-  
50 ties is obtained than has heretofore been possi-  
ble, and in which any detrimental and undesir-  
able features which might be attributed to the  
presence of such soaps or of a small amount of  
free oleic acid can be readily overcome by the  
55 addition of a suitable antioxidantizing agent such

as diphenylamine, resorcinol, phenol, or hydro-  
quinone.

Among the further objects of the invention is  
the provision of a method which comprises pro-  
tecting and lubricating fabric, yarn, thread, fila-  
60 ments, or textile fibres, artificial as well as nat-  
ural, during mechanical operations upon them  
and dyeing the said materials, which method does  
not require the removal of the lubricating and  
protecting agent from the said materials in a 65  
separate operation prior to contact of said ma-  
terials with dyeing agents. The invention may  
be applied to natural fibres, fabric, thread or  
yarn, such as cotton, silk, etc., or to artificial  
fabrics, yarn, threads, or filaments such as vis-  
70 cose silk, cellulose acetate silk, cuprammonia and  
nitro silks and the like, or mixtures thereof, elimi-  
nating the heretofore necessary step of scouring.

According to the present invention the fabric,  
yarn, thread or filament is impregnated with or  
75 has applied to it, in any suitable manner, a com-  
position consisting essentially of a mixture of  
suitable mineral oil lubricant, a suitable alkali  
metal soap-like emulsifying agent such as the  
sodium or potassium soap of oleic acid, trieth-  
80anolamine soap of oleic acid, and mahogany sul-  
fonates or mineral oil sulfonates such as may be  
obtained by treating crude mineral oil stocks  
or naphthas with concentrated or fuming sulfuric  
acid and reacting upon the obtained sulfonic 85  
acids with an alkali metal hydroxide such as so-  
dium hydroxide. These mineral oil sulfonates or  
mahogany sulfonates are well known and there-  
fore need no detailed description here. It is  
preferable, however, to employ purified sulfonates 90  
because of their lighter color and generally more  
acceptable operation. As sulfonates may also be  
used the alkali metal salts of the sulfonic acids  
obtained by allowing an excess of sulfuric acid  
to act upon an aromatic hydrocarbon, for exam-  
95 ple, naphthalene, or benzene, in the presence of  
oleic acid, such sulfonic acids being sometimes  
known as Twitchell reagent, and the term min-  
eral oil sulfonate as used herein is used as in-  
cluding these reagents as well as true mahogany 100  
or mineral oil sulfonates.

A further part of the present invention con-  
sists in utilizing in the above described compo-  
sition a free fatty acid, such as oleic acid, which  
is particularly useful to make the soaps used as  
described above dissolve completely and clearly—  
the probabilities being that the added free fatty  
acid counteracts hydrolysis of the soaps used. A  
still further part of the invention consists in  
adding to the mixture of mineral oil, soaps and 105  
110

mineral oil sulfonates, solvents for potassium soaps, which are as a rule difficult to prepare in the form of a clear solution, and for this purpose the following solvents may be used; mono-  
5 ethylether of diethyleneglycol (carbitol), mono-  
butylether of ethylene glycol (butyl cellosolve),  
monobutylether of diethyleneglycol (butyl car-  
bitol), etc.

As mineral oil any acid free, clear, colorless, or  
10 slightly colored mineral lubricating oil may be  
used. A chemically inert and stable mineral lu-  
bricating or paraffin oil from 30 seconds Saybolt  
viscosity (100° F.) up may be used. The viscos-  
ity of the oil may be even as high as 80 seconds  
15 Saybolt viscosity. However, a mineral oil with  
a viscosity between 30° and 70° Saybolt acts very  
satisfactorily. The so-called white oils, which  
are purified mineral lubricating oils, may be ad-  
vantageously employed as the mineral oil.  
20 The composition may be prepared by intimate-  
ly mixing the various ingredients in the desired  
proportions, and as examples of various composi-  
tions, ranges of proportions, and what are now  
believed to be preferred proportions, the follow-  
25 ing are given; but it is to be understood that the  
invention is not limited to these specific examples:

*Example 1*

| 30                                            | Preferred proportions | Ranges of proportions |
|-----------------------------------------------|-----------------------|-----------------------|
|                                               | Percent               | Percent               |
| Mineral oil #30.....                          | 60                    | 40-75                 |
| Sodium salt of mineral oil sulfonic acid..... | 9                     | 5-14                  |
| 35 Potassium oleate.....                      | 16                    | 5-20                  |
| Triethanolamine soap of oleic acid.....       | 9.7                   | 4-30                  |
| Oleic acid.....                               | 0.3                   | 0.1-4                 |
| Monoethylether of diethyleneglycol.....       | 5.0                   | 3-10                  |
| Diphenylamine.....                            | Trace.                | 0.01-0.1              |

*Example 2*

| 40                                            | Preferred proportions | Ranges of proportions |
|-----------------------------------------------|-----------------------|-----------------------|
|                                               | Percent               | Percent               |
| 45 Mineral oil #50.....                       | 65                    | 40-75                 |
| Sodium salt of mineral oil sulfonic acid..... | 8                     | 5-12                  |
| Potassium oleate.....                         | 13                    | 5-20                  |
| Triethanolamine soap of oleic acid.....       | 9.2                   | 4-30                  |
| Oleic acid.....                               | 0.3                   | 0.1-4                 |
| Monobutylether of diethyleneglycol.....       | 4.5                   | 3-10                  |
| 50 Resorcinol.....                            | Trace.                | 0.01-0.1              |

In practical use triethanolamine soap of oleic acid has proved to be very satisfactory, but the corresponding mono- and di-ethanolamine soaps may also be used. The latter two, however, may not be employed with like advantage as the former. An objection against the use of the mono- and di-ethanolamine soaps is that the elimination of soaping or scouring before dyeing, referred to herein, cannot be so well obtained and, furthermore, when using these soaps a larger proportion of free oleic acid would be necessary, and such larger proportions of oleic acid in the coning or winding oil described herein is not desirable. Monoamylamine soap of oleic acid gives very satisfactory results as a substitute soap for the triethanolamine soap, but its strong odor may prove an objection to some extent in commercial use.  
55 In preparing the composition when utilizing a solvent, for example monoethylether or butylether of diethylene glycol, as in Examples 1 and 2 it is preferable to dissolve the potassium soap of oleic acid (potassium oleate) in the solvent before mixing the ingredients together. The

solvents used should be water free or substantially water free, and the remaining ingredients likewise should also be substantially water free at the time the composition is made, if a clear product is to be prepared. Heat may be employed to bring the ingredients into solution.

Fabrics, yarn, threads and filaments which have been coated or impregnated with the composition of the present invention, either before or during the making of the fabric or other articles, may be passed into the dye bath or brought into contact with a dyeing liquid without preliminary hot soaping, scouring or similar treatment, to remove the winding oil composition or oil part thereof. The oil coating or impregnating of the fabric, yarn, threads, or filaments, on such direct entry of the oiled or lubricated material into a neutral or alkaline dye bath does not de-emulsify or break out as an oily liquid even when the dye bath contains inorganic salts added for the sake of better exhaustion of the dye bath. Examples of such inorganic salts are sodium chloride and sodium sulphate. Thus the oil or components thereof does not float on the top of the dye bath or prevent or decrease the dye absorption when the dye is in contact with the fabric, yarn or filament. The invention, therefore, also contemplates the dyeing of the fabric, yarn or filament without previous removal or substantial removal therefrom of the winding or coning oil composition by scouring.

In treating yarns, threads or filaments which weaken when wetted out, such as yarns, threads, or filaments of certain artificial materials, it is desirable that they be treated in the dry state with the composition also substantially free from water. Otherwise, the composition may be applied to the material to be treated while it is more or less in a wet condition and the composition applied to the material in this condition may or may not contain considerable water content. It is also within my invention to apply the composition substantially free of water to a substantially dry fabric, yarn, thread or filament for lubricating and protecting them during various operations to which they may be subjected in the textile industry, for example, weaving, knitting, braiding, winding or coning of threads or filaments.

Using an amine soap and alkali metal soap together in the composition as more fully set forth in Examples 1 and 2 above, has been found in practice to result in a composition of the character described with excellent properties as regards lubrication and protection, solubility or emulsifying power, stability, nonimpairment of the dyeing process, appearance and odor of the product, elimination of washing or scouring due to the rapid emulsification of the oil with water or salts containing dye bath, prevention of adhesion of wound fibre or yarn, moisture proofing, and general applicability for the purposes intended.

The compositions described herein are usually employed between the time the fibre is formed, for example fibres of viscose silk, and the time the final product, such as woven fabric or knitted goods or other article, is finished.

The terms "lubricating", "lubrication", or "lubricating power", used herein are used to describe the property of the composition or other material which protects the yarn threads or filaments by decreasing the friction between them and the machine parts with which they come in

80

85

90

95

100

105

110

115

120

130

135

140

145

150

contact and/or which decreases friction between yarn, threads, or filaments themselves.

I claim:

1. A process for treating natural and artificial threads, filaments, and the like which comprises applying to the said materials a composition including a mineral oil, a mineral oil sulphonate in such proportion as to be substantially ineffective with respect to the lubricating properties of the mineral oil, an additional emulsifying and lubricating agent including alkali metal and organic base soaps, and a solvent for the soaps, and thereafter without prior substantial removal of said composition from the said materials, dyeing the said materials.

2. A process for treating natural and artificial threads, filaments, and the like which comprises applying to the said materials a composition including a mineral oil, a mineral oil sulphonate, alkali metal and organic base soaps, and a solvent for the said soaps of the class consisting of monoethylether of diethyleneglycol and monobutylether of diethyleneglycol, and thereafter dyeing the said materials without prior substantial removal of the composition from the said materials.

3. A process according to claim 1, in which the said composition further includes oleic acid and an antioxidantizing agent.

4. A process for treating natural and artificial threads, filaments, and the like which comprises applying to the said materials a composition including a mineral oil, a mineral oil sulphonate, an alkali metal and triethanolamine soap of oleic

acid in such proportion that a slight excess of free oleic acid is maintained, a solvent for the said soaps, and thereafter dyeing the said materials without prior substantial removal of the composition from the materials.

5. A process for treating natural and artificial threads, filaments, and the like which comprises applying to the said materials a composition including 40 to 75% mineral oil, 5 to 14% mineral oil sulphonate, 5 to 20% potassium oleate, 4 to 30% triethanolamine soap of oleic acid, 3 to 10% monoethylether of diethyleneglycol, and thereafter dyeing the said materials without prior substantial removal of the composition from the materials.

6. A process for treating natural and artificial threads, filaments, and the like which comprises applying to the said materials a composition including 40 to 75% mineral oil, 5 to 12% mineral oil sulphonate, 5 to 20% potassium oleate, 4 to 30% triethanolamine soap of oleic acid, 3 to 10% monobutylether of diethyleneglycol, and thereafter dyeing the said materials without prior substantial removal of the composition from the materials.

7. A process according to claim 5, in which the said composition contains 0.1 to 4% free oleic acid.

8. A process according to claim 5, in which the said composition contains a slight excess of free oleic acid and a trace of an antioxidantizing agent of the class consisting of diphenylamine and resorcinol.

ALEIDUS G. BOUHUYS.

35

110

10

115

15

120

50

125

15

130

10

135

5

140

0

145

5

150

80

85

90

95

100

105

110

115

120

125

130

135

140

145

150